

May 28, 1935.

A. C. WEIERICH

2,002,806

METHOD OF PRODUCING ORNAMENTAL ENAMELED WARE

Filed July 30, 1932



INVENTOR  
Andrew C. Weierich  
BY Evans & McCoy  
ATTORNEYS

## UNITED STATES PATENT OFFICE

2,002,806

METHOD OF PRODUCING ORNAMENTAL  
ENAMELED WAREAndrew C. Weierich, Cleveland, Ohio, assignor to  
The Vitreous Enameling Company, Cleveland,  
Ohio, a corporation of Ohio

Application July 30, 1932, Serial No. 626,581

16 Claims. (Cl. 41—24)

My invention relates to enameled ware, and more particularly to a method of producing ornamental enameled ware.

The principal object of my invention is to provide an article of ornamental enameled ware in which a vitrifiable material, such as enamel, is applied to a metal in such a manner that a highly ornamental effect is obtained.

A further object of my invention is to provide a process of producing ornamental enameled ware, in which enamel in the form of globules or lumps is projected upon ware having a ground coating, or a ground and base coating, thereon, in such a manner that a pleasing effect will be produced.

A still further object of my invention is to provide a process of producing enameled ware, in which an embossed enamel design is applied in the form of lumps or globules upon an enameled base or ground coating of a different color, and a coating of enamel having a still different color is sprayed at a lateral angle against the enamel design, thereby shading one side of the design and causing an intermingling of the colors of the base coat and the shading coat to provide an illusionary color effect.

In the accompanying drawing,

Figure 1 is a fragmentary perspective view of a sheet of ornamental enameled ware produced by my improved process;

Fig. 2 is an enlarged cross-sectional view of a portion of the sheet shown in Fig. 1 before the burning operation;

Fig. 3 is a perspective view of coated enameled ware showing the method of applying the design; and

Fig. 4 is a perspective view showing the method of applying the shading coat.

In producing ornamental enameled ware, it has heretofore been the practice to apply a ground coating, or a ground and a base coating, and while the ground or base coating is still wet to spray or otherwise project small globules of the same or different colored enamel upon the ground or the base coating. In such practice, however, the drops or globules of enamel sink into the ground or the base coating and a distinctive embossed design is not produced.

By my invention I have provided a process of producing ornamental enameled ware having an embossed design of a highly pleasing appearance. In practicing my invention, a ground coating is first applied to the metal ware which is usually formed of sheet iron, cast iron, or steel. This may be performed in the usual manner, such as

by dipping or spraying. The ground coating is then dried and burned, or preferably just dried, and the same or a different colored enamel is projected on the ground coat in the form of lumps or globules. In the event that the ground coating is both dried and burned, the ware must be first heated before applying the drops or globules, so that when the drops or globules hit the warm surface they dry immediately in round lump form.

I preferably utilize a spray having a very low air pressure for projecting the lumps or globules upon the ground coating. The lumps may be sprayed on the dried ground coating in the form of any appropriate design or configuration and, if desired, a stencil having openings corresponding in shape to the design may be placed over the dried ground coat and the lumps sprayed, or otherwise projected, through the openings in the stencil.

It will be particularly noted that in practicing my invention the ground coating is first dried before the ornamental design is applied; otherwise, the lumps will have the tendency to sink into the ground coating instead of protruding therefrom. After the ornamental design is applied, the coated ware may be burned to vitrify the enamel in the usual manner.

The enamel is burned at a temperature of approximately 1450° to 1600° F., the particular temperature depending upon the composition of the enamel and the time of firing. During the burning operation the heat is sufficient to cause the enamel of which the lumps are composed to become viscous and to adhere to the ground coat. The temperature and time of firing, however, should not be sufficient to cause the applied lumps to become so liquid that the desired contour of the projected lumps or globules will be affected.

Instead of applying the design in the form of lumps or globules directly upon the ground coating, I preferably first apply a ground coating, dry and burn the ground coating, and then apply a thin base coating of enamel which is also dried. The ornamental design is then sprayed or projected in the form of lumps or globules upon the dried base coating.

The globules or lumps may be projected in any desired design upon the prepared surface. I preferably utilize a stencil for this purpose and project the lumps or globules through openings in the stencil or, if desired, the drops or globules may be projected over the entire surface, a stencil applied, and the unburned enamel that is exposed through openings in the stencil brushed away.

In the latter case, it is of course necessary that the foundation metal shall be first previously provided with a burned coating. The applied lumps may also be shaded with a different colored coating before the stencil is applied or after it has been removed. It will also be understood that it is not necessary to utilize a stencil as portions of the lumps may be removed in any desired manner. Instead of applying a coating, 10 burning the applied coating and applying an additional coating which is only dried, the layer of enamel in the form of globules or lumps may be applied to the burned coating. In such cases, however, it is necessary that the foundation 15 metal shall be hot during the application of the coating which is in the form of lumps or globules so that they will dry in round lump form.

When both a ground and a base coating are applied, it is necessary to burn the ground coating before the base is applied, as is the usual 20 practice. As in the previous example, the base coating should also be thoroughly dried before applying the design so that the lumps or globules forming the design will not sink into the base 25 coating.

After the embossed designs have been applied, a highly ornamental effect may be produced by spraying a different colored enamel against the 30 sides of the lumps from a substantially lateral direction. The shading produced causes the embossed design to stand out in a distinctive manner, which adds to its natural beauty.

In preparing ornamental enameled ware, a 35 pleasing effect may be produced by first applying a ground coat which is dried and burned. A thin base coat of a light colored enamel, such as a white colored enamel, is next applied. The base coat is then thoroughly dried and a design 40 formed of a different colored enamel, such as yellow, is projected in the form of globules or lumps upon the dried base coating. The design is preferably applied through openings in a stencil, although this is not essential. If a stencil is utilized, it is then removed and a coating having 45 a different color, such as brown, is sprayed laterally against the one side of the embossed design. The brown coating upon being sprayed against the yellow lumps, produces a design having a shaded appearance and also provides a thin brown coating over the white base coating. The 50 brown coating, however, is not sufficient to completely obscure the white color. The thin brown coating upon the white base coating causes an intermingling of colors, producing an illusionary 55 effect, so that the color between the projected designs appears as if a lavender colored base coating has been applied, and the design projected upon the lavender base coating. The 60 enameled coatings which have been applied are then burned in the usual manner.

Another combination of coatings which I have 65 found particularly desirable, may be produced in the following manner. The usual ground coat is first applied in any suitable manner, such as by dipping or spraying. The ground coat is then dried and burned. A white base coating is next applied and thoroughly dried. A stencil is then placed over the dried base coating and drops or 70 globules of a green colored enamel are projected through openings in the stencil. An embossed design of a green colored enamel is thus provided upon a white base coat. A black colored 75 enamel is then sprayed from a lateral direction against the green lumps, shading the lumps on one side and forming a thin coating over the

white colored enamel in the spaces which were covered by the solid portion of the stencil. The thickness of the black coating, however, is not sufficient to completely obscure the white base coating, and the intermingling of the white and black colors produces an illusionary effect having a lavender colored appearance. The embossed green projections prevent the laterally sprayed black coating from covering the white base coating immediately adjacent the projections on the opposite side to that which is shaded. After the 10 coatings have been applied, they are burned to vitrify the enamel. It will thus be seen that such a combination of coatings produces a lavender background with a projecting green design which 15 has a black border on one side and a white border on the other.

Instead of projecting the embossed design in the form of globules or lumps upon the ground or base coating, a light colored ground coating may 20 be applied and dried, or a ground coating may be applied, dried and burned, and a base coating applied and dried. A thin coating of a darker colored enamel may then be sprayed from a substantially lateral direction against the light colored ground or base coating. The spraying of the dark colored enamel from a lateral direction on the dry enamel builds up small lumps of the dark colored enamel. The intermingling of the light colored base and the superposed darker colored coating which is laterally applied, produces an enameled article which appears as if projecting lumps had been applied and shaded, whereas the enamel is substantially smooth. The applied 25 coatings are then burned in the usual manner.

Enameled ware having a border formed by the method described in the preceding paragraph and a central portion formed of embossed shaded lumps may be readily formed and a pleasing ornamental effect obtained in the manner illustrated in the accompanying drawing. It will be understood, however, that the drawing is merely 30 illustrative, as I do not desire to limit myself to the particular colors, structure and process disclosed therein.

Referring to the drawing, a sheet of metal 1, such as iron, cast iron, or steel, is first dipped or otherwise provided with a suitable ground coat 2. The ground coat is dried and burned. A thin layer of a light colored base coat 3, such as white, 40 is next applied, which is also dried. A stencil 4 is then preferably placed over the central portion of the coated enamel ware and globules or lumps of a green colored enamel are projected through openings in the stencil. This may be 45 conveniently accomplished by means of a low pressure spray. If desired, the border may also be sprayed with a thin coating of green by the usual spraying process, a low pressure spray not being required for this purpose. The stencil is then 50 removed. The ware is thus provided with a green embossed design 5, a green border 6 and white colored spaces between the design formed by that portion of the base coat which was covered by the solid portion of the stencil when the design 55 was applied. A dark colored enamel, such as black, is then sprayed in a lateral direction against the lumps. The dark enamel provides a thin covering over the white spaces between the embossed designs and is projected against the green coating forming the border. This coating is not of sufficient thickness to completely obscure the 60 white base coat between and around the designs. The black coating superimposed upon the white coating produces an illusionary effect and the 65 70 75 75

spaces between the designs really appear as if a base coating of enamel having a lavender color was applied. The thin black coating sprayed from a lateral direction upon the green border forms 5 a coating having the appearance of projecting green lumps, whereas in reality the border is substantially smooth. In spraying the black coating against the embossed design, the downwardly extending portion of one side of the embossed de- 10 sign and one side of each projecting lump will be shaded, as indicated at 1. The white base coating immediately adjacent the opposite side of each of the embossments, however, will be protected from the black coating. The embossments 15 are thus provided with a black shading on one side and a white border 8 on the opposite side. The embossments will therefore be clearly defined and will have the appearance of projecting a greater distance from the base than they really 20 do.

It will be understood that when both a ground and a base coating are applied, it is necessary to both dry and burn the ground coating before applying the base coating. Before applying the 25 globules or lumps, however, the base coat is preferably only dried and not burned. If it is burned it is necessary to heat it before applying the globules or lumps. It is therefore apparent in the specification and claims that where drying is mentioned before applying the globules or lumps, the 30 equivalent step of drying, burning and heating the burned coating before applying the globules or lumps may be utilized.

From the foregoing description it will be seen 35 that I have produced ornamental enameled ware which is distinctive in design and pleasing in appearance, and which is capable of being produced in a simple and economical manner. My improved method is also exceptionally novel in that 40 a design of any desired configuration may be provided and since the ground or base coating is first thoroughly dried before the embossed enamel designs are applied, the design will project from the surface in a distinctive manner.

45 The shading also aids in sharply defining the projecting design and gives it a distinctive appearance. By shading the embossed portions and at the same time providing a thin dark colored coat over the spaces between the designs and 50 upon the border coating, a varicolored design may be produced in an economical manner.

It will be understood that while I prefer to utilize a combination of distinctive features in 55 providing my improved design, each of the distinct features in and by itself represents an advance in the art. In particular, the step of first drying the base coating before applying the globules or lumps to form the design is especially desirable, because it prevents the applied lumps or 60 globules from penetrating into the base coat. A highly distinctive design is thus obtained which, together with the shading and color combination produced by my improved method, enables the 65 production of ornamental enameled ware having a pleasing appearance.

To those skilled in the art, many modifications of and widely differing embodiments and applications of my invention will suggest themselves without departing from the spirit and scope thereof. My disclosures and the description herein are 70 purely illustrative and are not to be in any sense limiting.

What I claim is:

1. The process of producing ornamental enameled ware which comprises applying an enamel 75

ground coating upon a foundation metal, drying the ground coating and then projecting globules or lumps of an enamel in the moist state upon the dried ground coating to form an ornamentation which projects from the surface of the ground coating, and then burning to vitrify the enamel and to provide projections which extend above the ground coating. 5

2. The process of producing ornamental enameled ware which comprises applying an enameled ground coating upon a foundation metal, drying and burning the ground coating and then projecting globules or lumps of an enamel in the moist state upon the burned ground coating while the foundation metal is hot to form an ornamentation 10 which projects from the surface of the ground coating, and then burning to vitrify the enamel and to provide projections which extend above the ground coating. 15

3. The process of producing ornamental enameled ware which comprises applying an enamel coating to a foundation metal, drying and burning the applied coating, applying a thin layer of an additional coating, drying the additional coating, projecting a coating in the form of moist 20 lumps or globules on the dried coating, drying the lumps, brushing away a portion of the lumps or globules, and then burning to produce enamelware having a projecting design. 25

4. The process of producing ornamental enameled ware which comprises applying an enamel ground coating upon a foundation metal, drying and burning the ground coating, applying a thin 30 layer of a base coat, drying the base coat, projecting globules or lumps of enamel in the moist 35 state on the dried base coat, and then burning to vitrify the enamel and form a base coating having projecting globules or lumps. 40

5. The process of producing ornamental enameled ware which comprises applying a ground 45 coating upon a foundation metal, drying and burning the ground coating, applying a thin layer of base enamel over the ground coating, drying the base coating, spraying a thin layer of a different colored enamel in a substantially lateral direction over the dried base coating to form 50 a substantially smooth surface which appears as if small lumps had been projected upon the base coating, and burning the final coating to produce enamelware having the appearance of a projecting design. 55

6. The process of producing ornamental enameled ware, which comprises applying a ground coating of enamel upon a foundation metal, drying and burning the ground coating, applying a 55 thin layer of an enamel base coating and drying the same, placing a stencil over the dried base coating, projecting enamel in the form of moist globules or lumps through the openings in the stencil, removing the stencil, and burning to produce enamelware having a projecting design. 60

7. The process of producing ornamental enameled ware, which comprises applying a ground coating of enamel upon a foundation metal, drying and burning the ground coating, applying a 65 base coating over the foundation metal, drying the base coating, projecting globules or lumps of enamel over the surface of the base coating, spraying a different colored enamel in a lateral direction against the surface of the applied lumps, 70 and finally burning the enamel to produce enamelware having a projecting design. 75

8. The process of producing ornamental enameled ware, which comprises applying a ground coat of enamel upon a foundation metal, drying

and burning the ground coating, applying a thin base coating of enamel over the ground coating, drying the base coating, placing a stencil over the dried base coating and projecting enamel in the form of lumps or globules through openings in the stencil to form projections, spraying a different colored enamel in lateral directions against one side of the projections, and then burning to vitrify the enamel and produce enamelware having a projecting design.

9. The process of producing ornamental enameled ware, which comprises applying a ground coat of enamel upon a foundation metal, drying and burning the ground coating, applying a thin light colored base coating of enamel over the ground coat, drying the base coat, applying a stencil over the dried base coat, projecting globules or lumps of enamel having a different color than the base coat through openings in the stencil upon the dried base coat to form an embossed design, removing the stencil, spraying a dark colored enamel in a substantially lateral direction against the sides of the lumps so as to form a dark colored coating upon one side of the embossed design and a thin layer over the base coating between the designs, and burning the enamel to vitrify the same and produce enamelware having a projecting design.

10. The process of providing ornamental enameled ware, which comprises applying a ground coating of enamel upon a sheet of metal, drying and burning the ground coating, applying a light colored base coating of enamel over the ground coating, drying the base coating, applying a stencil over the central portion of the sheet, thereby partially covering the base coat, projecting globules or lumps of enamel having a different color through the openings in the stencil to form an embossed design, removing the stencil and spraying a dark colored enamel in a substantial lateral direction against the sides of the design so as to form a dark colored coating on one side of the embossed design, a thin dark layer over the base coating between the projections forming the design to produce an illusionary effect, and a substantially smooth coating over the border which has the appearance of being applied in the form of small lumps, and burning the enamel to vitrify the same and produce enamelware having a projecting design.

11. The process of producing ornamental enameled ware which comprises applying an enameled coating to a foundation metal, drying and burning the applied coating, applying a thin layer of an additional coating, drying the additional coating, projecting a coating in the form of lumps on the dried coating, spraying a coating in a lateral direction against the lumps to produce a

shaded effect, burning to produce enamelware having a projecting design, applying a stencil over the shaded lumps and brushing away the unburned enamel exposed through the openings of the stencil.

12. The process of producing ornamental enameled ware which comprises applying an enameled coating to a foundation metal, drying and burning the applied coating, applying a coating in the form of lumps on the burned coating while the metal is hot, drying the lumps and brushing away a portion of the lumps, and then burning the enamel to produce enameled ware having a projecting design.

13. The process of producing ornamental enameled ware which comprises applying a ground coating upon a foundation metal, drying the ground coating, spraying a thin layer of a different colored enamel in a substantially lateral direction over the dried base coating and then firing to produce a substantially smooth coating having the appearance of being applied in the form of small lumps.

14. The process of producing ornamental enameled ware which comprises applying a ground coating upon a foundation metal, drying and burning the ground coating, heating the metal, spraying a thin layer of a different colored enamel in a substantially lateral direction over the ground coating, and then firing to produce a substantially smooth coating having the appearance of being applied in the form of small lumps.

15. The process of producing ornamental enameled ware which comprises applying a ground coating upon a foundation metal, drying and burning the ground coating, applying a base coating, drying and burning the base coating, heating the metal, then spraying a different colored enamel in a substantially lateral direction over the base coating to form a substantially smooth surface which appears as if small lumps had been projected upon the base coating, and burning the final coating to produce enamelware having the appearance of a projecting design.

16. The process of producing ornamental enameled ware which comprises applying a ground coating upon a foundation metal, drying and burning the ground coating, applying a thin layer of base enamel over the ground coating, drying the base coating and spraying a thin layer of a different colored enamel in a substantially lateral direction over the dried base coating to form a substantially smooth surface which appears as if small lumps had been projected upon the base coating, and then burning to vitrify the enamel, and then burning the final coating to produce enamelware having the appearance of a projecting design.

ANDREW C. WEIERICH.